

## UNITED STATES PATENT OFFICE

2,039,327

## PEN POINT

Hiram Stanhope Lukens, Philadelphia, Pa., assignor to C. Howard Hunt Pen Company, Camden, N. J., a corporation of New Jersey

No Drawing. Application May 13, 1935,  
Serial No. 21,189

1 Claim. (Cl. 120—109)

This invention relates to pen points, and the invention is especially concerned with a novel type of gold plated pen point.

Heretofore, it has been quite common to employ solid gold pens or nibs in fountain pens, and solid gold pens of this type have certain advantages, particularly with respect to corrosion resistance, smoothness of ink flow, and appearance. These pens, however, must obviously be relatively expensive, and the present invention has in view the provision of a relatively inexpensive pen point having the advantages of the solid gold type of pen.

For this purpose I prefer to make my improved pens from a chromium alloy steel, such as the so-called corrosion resistant steel alloys which are usually chiefly comprised of chromium, nickel and iron, and to apply a gold plate thereon by electrodeposition. Corrosion resistant alloys of the type in question may also contain smaller amounts of other ingredients added for the purpose of improving the corrosion resistance and other properties of the product. An alloy which I find especially suitable for pens is one containing about 18% chromium, about 8% nickel and about 2½% molybdenum. By gold plating such an alloy I am enabled to secure a high degree of acid resistance, smoothness of ink flow and also gold appearance. Furthermore, my improved pen, being made of a very tough alloy steel, is very durable and not readily damaged or worn.

In considering the nature of this invention, especially the manner in which my pen is rendered substantially corrosion proof and acid resistant, it should be borne in mind that all plating, applied as by electrodeposition, is porous. In view of this, if the base metal on which the plating is deposited is subject to attack by acid ingredients in ink, the plated pen would also be subject to such attack, the rate of attack being only very slightly reduced by the presence of the porous plating. However, the base metal of my improved pen is of a corrosion proof or acid resistant nature, because of the oxide film which normally forms on such alloys, so that even though the gold plating (which, as will herein-after appear, is applied to the oxide film) is porous, the pen is not subject to attack by acids.

It should further be noted that considerable difficulty has been encountered in the past in satisfactorily applying a plating of the type here in question to alloy steels of the so-called "stainless" type which are characterized by the formation of an oxide film on the exposed surfaces.

This difficulty resulted from several causes, one of which is probably the fact that the oxide film which forms under usual or normal conditions, is of a spongy, friable or fragile nature. In any event, this normal type of oxide film does not adhere tenaciously to the metal, so that attempts to apply a plate thereon have been unsuccessful. The plating of such attempts, in fact, is so lacking in adherent properties, that even slight rubbing, as with a finger, is frequently sufficient to remove the deposited metal. I have also found that the usual type of gold plating solutions employed in many industries are unsuccessful in applying an adherent gold plating, probably because of the alkalinity of the usual gold plating solution which apparently has the effect of even further increasing the spongy and non-adherent nature of the oxide film almost immediately upon immersion of the articles into the plating solution.

With the foregoing factors in mind, I first form the pens from a suitable chromium alloy steel, such as that referred to above, and then subject the pens to a treatment to produce a tough, dense and highly adherent oxide film thereon. Nitric acid may be employed for this purpose and the acid may be used either to toughen the relatively spongy and non-adherent film normally present on the alloy or to produce a new film (after removal of the usual spongy film), which new film also is of a highly adherent character. The acid may be used in concentrated form or in a solution containing as low as 5%, or even lower, although the time of treatment must be increased with the low concentrations. Ordinarily from about 5 to 10 minutes in a solution containing upwards of 10% nitric acid will be found to be sufficient.

Following this treatment, I immerse the pens in a plating bath containing free hydrocyanic acid. This may be accomplished by employing a bath containing the following ingredients in about the proportions indicated:

|                                |       |        |     |    |
|--------------------------------|-------|--------|-----|----|
| Concentrated hydrochloric acid | ----- | pint   | 1   | 45 |
| Sodium cyanide                 | ----- | ozs.   | 8   |    |
| Sodium gold cyanide            | ----- | oz.    | 1/8 |    |
| Water                          | ----- | gallon | 1   |    |

I have found that the presence of free hydrocyanic acid is an important factor in providing an adherent deposit. The quantity of this acid present is not critical. Preferably the bath should contain sufficient to give a slight acid reaction to litmus, and the quantity may be carried up at least to an amount equivalent to that which will

- combine with the gold present. Having initially prepared a bath with the proportions of ingredients listed above, I prefer to renew the supply of hydrocyanic acid either by adding an additional supply of sodium cyanide at periodic intervals or in some other equivalent manner. As a guide in determining when additional sodium cyanide is necessary, the brilliance of the deposit may be observed. When the deposit noticeably loses its brilliance, additional cyanide should be added. Ordinarily, in the average plating bath of fifteen gallons capacity, it is sufficient to add a few ounces of sodium cyanide for each 500 gross of pens plated.
- 15 It is of importance in this process to ensure that the plating commences immediately upon immersion of the articles in the plating solution, this, apparently, for the reason that the nature of the plating bath is such as tends to destroy or 20 impair the toughness and adherence of the oxide

film. With this in mind, the cathode connection should be made or completed to the article being plated prior to immersion of the article in the bath.

Following the first deposit of gold, I prefer to apply an additional gold plate which may conveniently be done in the more usual type of plating solution containing, for example,  $\frac{1}{2}$  ounce sodium gold cyanide, and  $2\frac{1}{2}$  ounces sodium cyanide per gallon of water.

10 Attention is directed to the fact that the method herein disclosed is also disclosed and claimed in my copending application Serial No. 21,190, filed May 13, 1935.

15 I claim:

A pen point composed of a chromium alloy steel having a dense and adherent oxide film thereon and further having an adherent electrolytically deposited gold plate applied to said film.

HIRAM S. LUKENS. 20